

## UNITED STATES PATENT OFFICE

2,279,830

## METAL PLATING BATH AND METHOD OF PLATING

John J. Murray, Arlington, Mass.

No Drawing. Application March 9, 1938,  
Serial No. 194,967

8 Claims. (Cl. 204—51)

This invention relates to a metal plating bath and particularly to a method of plating chromium.

At the present time the most widely employed chromium plating bath is one utilizing, in addition to chromic acid, a solution of a sulfate. Such solutions require constant regulation and work only with narrow ranges of  $\text{SO}_4$  ion concentration and are very low in efficiency.

In accordance with the present invention a plating solution of relatively high plating efficiency, of considerable stability and one not requiring regulation, is produced.

In accordance with this invention, a halogen derivative of acetic acid, preferably monochloracetic acid, is employed in combination with chromic acid.

The relative concentrations of chromic acid and monochloracetic acid may be widely varied. Preferably, 5% of monochloracetic acid is used based on the chromic acid because at this ratio make-up chromic acid may be added from time to time in the same relative proportion to monochloracetic acid. However, much higher concentrations may be employed as, for example, 9 oz. of monochloracetic acid to 36 oz. of chromic acid, or as little as 1% may be employed. At the higher concentrations the plating is heavier and the solution tends to heat more rapidly. At the lower concentrations the plating is not so heavy.

A preferred plating bath comprises, to each gallon of water 36 oz. of chromic acid and 2 oz. of monochloracetic acid. With such a bath, it is preferable to use a lead electrode. The solution may be run hot or cold, but is preferably run from 90° to 130° F. The current density may be widely varied. For example, a current density of 1,000 amperes to 9 square feet is satisfactory, whereas, in other instances 2,000 amperes have been employed for 27 square feet. Plating efficiencies as high as 37% have been procured.

Using a current density of 1,000 amperes for 9 square feet and the above bath containing 36 oz. of chromic acid to 2 oz. of monochloracetic acid, the deposit on a square foot is approximately .0003" in five minutes. This uses up approximately  $\frac{1}{2}$  oz. of chromic acid and a corresponding amount of monochloracetic acid. Accordingly, make-up is added periodically in the original ratio of 36 to 2 and the process may be operated for months without any analysis, by making it up in this manner.

For the brighter chromium finishes, it is preferred to keep the current density lower, for example, plating only .00015 in four minutes.

In the bath herein described, chromium plating may be carried on successfully without the critical re-cleaning operations necessary heretofore. In fact, even the presence of tallow will not seriously interfere and metal may be introduced to

the bath without any previous cleaning whatsoever, if desired.

The dichloracetic acid and trichloracetic acid, while operating satisfactorily, are more expensive and are more corrosive to the hands. These are likewise used around 5%.

Metallic chromium produced in the layers by this process has a considerably different appearance than the ordinary electrolytic chromium. It has a more metallic look, is heavy, less brittle, and is not full of cracks.

The solution may likewise be used to plate lead, employing a lead nitrate bath. For example, in one gallon of water saturated with lead nitrate 10 16% of glycerin and 5% of monochloracetic acid are employed based on the lead. A low current density is employed and the bath is preferably cold.

The use of monochloracetic acid likewise increases the efficiency of a copper plating bath 15 and produces a copper film which has considerable strength and the color of which resembles that of copper produced by cooling from fusion.

The foregoing detailed description has been 20 given for clearness of understanding only, and no unnecessary limitations should be understood therefrom, but the appended claims should be construed as broadly as permissible in view of the prior art.

30 I claim:

1. A chromium plating bath comprising chromic acid and a minor proportion of a chlorinated acetic acid.

2. A chromium plating bath comprising chromic acid and a minor proportion of monochloracetic acid.

3. A plating bath comprising approximately 1 gallon of water, 36 oz. of chromic acid and 2 oz. of monochloracetic acid.

4. A plating bath comprising water, chromic acid and monochloracetic acid, the monochloracetic acid being 1 to 25% of the chromic acid by weight.

5. A process for electroplating chromium, which comprises passing an electric current from an anode to a cathode through an aqueous solution of chromic acid and monochloracetic acid.

6. The method as set forth in claim 5, in which the bath comprises approximately 1 gallon of water, 36 ounces of chromic acid and 2 to 9 ounces of monochloracetic acid.

7. The method as set forth in claim 5, in which the bath comprises water, chromic acid and monochloracetic acid in the proportion of 1 to 25% of chromic acid by weight.

8. The method of plating chromium which comprises passing an electric current through an electrolyte solution comprising chromic acid and a minor proportion of a chlorinated acetic acid.

JOHN J. MURRAY.